

## 1

3,689,258

## LOW CARBON HIGH TENSILE STRENGTH ALLOY STEEL

Joseph R. Zanetti, Dearborn, Mich., assignor to  
National Steel Corporation

No Drawing. Original application Aug. 11, 1967, Ser. No. 659,885, now Patent No. 3,544,393, dated Dec. 1, 1970, Divided and this application July 14, 1970, Ser. No. 62,734

Int. Cl. C22c 39/14

U.S. Cl. 75—126 F

3 Claims

### ABSTRACT OF THE DISCLOSURE

A low carbon, weldable, high tensile strength alloy steel characterized by ductility and toughness suitable for structural uses is produced in the "as rolled" condition by utilizing a steel consisting essentially, by weight, of

|           | Percent, about |
|-----------|----------------|
| Carbon    | .10-.20        |
| Manganese | .75-1.15       |
| Silicon   | .50-1.0        |
| Chromium  | .50-.80        |
| Zirconium | .05-.20        |
| Boron     | .0005-.0025    |
| Titanium  | .02-.15        |
| Columbium | .01-.06        |

and the balance iron with residual impurities. The steel is hot rolled to form bars, plate and sheets with a starting rolling temperature between 2100° F.-2300° F. and a finishing rolling temperature between 1400° F.-1700° F. followed by air cooling.

This invention is a division of copending application Ser. No. 659,885, filed Aug. 11, 1967, which is concerned with low carbon, high tensile strength, alloy steel. More specifically it is concerned with low carbon, high tensile strength, alloy steel having a minimum tensile strength of about 75,000 p.s.i. in the "as rolled" condition.

Low carbon, high tensile strength steels of the prior art have required heating, quenching, and tempering treatments subsequent to rolling in order to develop the desired tensile strengths and suitable ductility and toughness. Such treatments require multiple and uneconomical handlings e.g. the product must be held rigidly to prevent warping while being cooled rapidly from a temperature about 1750° F., and higher, to room temperature in about 10 to 25 seconds.

The quenching develops 100% marsteinic steel and is required to obtain desired high tensile strength. Without such quench treatment, such steels have a tensile strength of about 50,000 to 60,000 p.s.i. in the "as rolled" condition.

After quenching, such steels previously required a tempering treatment at about 850° F. to about 1300° F. to develop ductility and other properties necessary for end product usage.

This invention provides an alloy steel with high tensile strengths in the range of about 80,000 to about 120,000 p.s.i. (minimum yield strength of 75,000 p.s.i.). In addition, the steel exhibits ductility and yield point elongation values suitable for normal fabrication of high tensile strength steels and toughness suitable to withstanding normal stresses encountered in use of such steels. Obtaining these results without treatment subsequent to rolling is one of the highly unexpected contributions of the invention.

The low carbon high tensile strength alloy steel of the present invention consists essentially of the following weight-percentages:

## 2

Percent, about

|                           |             |
|---------------------------|-------------|
| Carbon                    | .07-20      |
| Manganese                 | .75-1.15    |
| Silicon                   | .50-1.0     |
| 5 Chromium                | .50-.80     |
| Zirconium                 | .05-.20     |
| Boron                     | .0005-.0025 |
| Titanium, about .15% max. |             |
| Columbium                 | .01-.06     |

10 the balance being iron with residual impurities such as are ordinarily encountered in conventional basic oxygen, open hearth, or electric furnace practice used in producing the steel. The maximum desirable values of the most common residual impurities encountered are:

|               |     |
|---------------|-----|
| 15 Phosphorus | .04 |
| Sulphur       | .05 |
| Copper        | .35 |
| 20 Aluminum   | .07 |

25 The upper limit of carbon is ordinarily not exceeded in order to maintain the good weldability of end product provided by the invention. Carbon content below the lower limit is ordinarily avoided in order to have sufficient carbon available for providing desired tensile strength.

30 The manganese is added in the furnace or the ladle. Where possible, e.g. in open hearth practice, it is added in both the furnace and the ladle. Preferably, the manganese is maintained in the range of .85% to 1.0% with a specific value of .90% being desired. The manganese helps increase the yield point and tensile strength of the steel and aids cold formability.

35 Silicon acts as a deoxidizer and ferrite strengthener. It can be added in the furnace or ladle; where possible silicon is added in both. Silicon is desirably kept in the range of .75% to .90% with .85% being preferred.

40 The chromium is added in the ladle and acts to increase both the yield point and tensile strength of the steel. A preferred specific value for the chromium is .65%.

45 The zirconium acts to increase hardenability, refine grain structure, increase toughness and cold formability. It is added in the ladle and is preferably kept between .075% and .12%; with .08% being the specific value aimed for.

50 The boron is added in the ladle. It increases hardenability of the steel and seeks out remnants of nitrogen in the steel to a greater extent than other nitride formers such as chromium, zirconium, columbium. The titanium helps to protect the boron for this purpose because of its greater affinity for oxygen than boron. A preferred value for the boron is .0010% and a preferred range is .0005% to .012%. The titanium also acts as a carbide former and is preferably kept at about .03%. The titanium should be added with the boron.

55 Columbium contributes to a number of the unexpected results obtained through the invention. It raises the yield point significantly without detrimental effect on the highly desirable ductility and toughness obtained by the invention in the "as rolled" condition. The columbium is added in the ladle, or can be added in the mold. A preferred specific value for the columbium is .035% and the preferred range is .035% to .06%.

60 65 If the steel is degassed during processing the ladle additions are made after degassing to minimize oxidation products and reduce possible contamination of the steel.

70 The alloy steel of this invention is rolled into bars, plate or sheets which are suitable for structural uses, railway car framing, and the like. This steel is characterized by high tensile strength, good weldability, high energy absorption capacity, and good ductility and yield point

elongation values in the "as rolled" condition. Data on these properties are set forth in the representative examples below:

EXAMPLE #1.—LOW CARBON COLUMBIUM TREATED ALLOY STEEL BARS HAVING A MINIMUM YIELD STRENGTH OF 75,000 p.s.i.

Dimensions:

.518" x .250 x 100"  
4½" x .312 x 110"

|                   | C   | Mn  | P    | S    | Si  | Cr  | Zr  | B     | Ti  | Cb   |
|-------------------|-----|-----|------|------|-----|-----|-----|-------|-----|------|
| Ladle chemistry   | .17 | .94 | .013 | .010 | .90 | .74 | .08 | .0012 | .03 | .038 |
| Recheck chemistry |     |     |      |      |     |     |     |       |     |      |
| (gauge):          |     |     |      |      |     |     |     |       |     |      |
| .250.....         | .17 | .94 |      |      | .87 | .75 | .09 | .0014 | .03 | .035 |
| .312.....         | .17 | .97 |      |      | .88 | .76 | .10 | .0014 | .03 | .037 |

MECHANICAL PROPERTIES

| Bars             | YS<br>(p.s.i.) | TS<br>(p.s.i.) | Elongation,<br>percent |                  | Bend  |
|------------------|----------------|----------------|------------------------|------------------|-------|
|                  |                |                | inches                 | Bend             |       |
| "As rolled"..... | 2% offset..... | .....          | 2-4-8 inches.....      | .....            | ..... |
| .250 gauge:      |                |                |                        |                  |       |
| Front.....       | 88,550         | .....          | 110,620                | 29-21-15 SB..... | ½ x T |
| Middle.....      | 78,100         | .....          | 106,930                | 29-21-16 SB..... | ½ x T |
| Back.....        | 80,540         | .....          | 111,360                | 24-16-11 SB..... | ½ x T |
| .312 gauge:      |                |                |                        |                  |       |
| Front.....       | 103,760        | .....          | .....                  | .....            | ..... |
| Middle.....      | 81,690         | .....          | 107,180                | 28-17-14 SB..... | ..... |
| Back.....        | 79,190         | .....          | 105,140                | 30-22-16 SB..... | ..... |

CHARPY "V" IMPACT TEST DATA

[Ft.-lbs.-at temperature ° F.]

| Thickness  | Direction         | Room<br>tem-<br>pera-<br>ture | Room<br>tem-<br>pera-<br>ture |      |      |     |     |
|------------|-------------------|-------------------------------|-------------------------------|------|------|-----|-----|
|            |                   |                               | 32                            | 0    | -20  | -40 | -60 |
| .250"..... | Transverse.....   | 12.7                          | 9.0                           | 6.7  | 4.8  | 3.0 | 2.2 |
|            | Longitudinal..... | 24.3                          | 17.7                          | 13.8 | 13.8 | 6.0 | 4.2 |
| .312"..... | Transverse.....   | 18.7                          | 10.7                          | 6.5  | 4.5  | 2.8 | 2.7 |
|            | Longitudinal..... | 39.0                          | 18.0                          | 12.3 | 6.0  | 3.8 | 3.2 |

EXAMPLE #2

|                      | C   | Mn  | P    | S    | Si  | Cu  | Cr  | Zr  | Al   | B     | Ti  | Cb   |
|----------------------|-----|-----|------|------|-----|-----|-----|-----|------|-------|-----|------|
| Ladle chemistry..... | .17 | .92 | .010 | .024 | .78 | .03 | .70 | .06 | .041 | .0007 | .03 | (0)  |
| Recheck chemistry:   |     |     |      |      |     |     |     |     |      |       |     |      |
| .250 gauge.....      | .18 | .90 | .009 | .025 | .79 | .04 | .70 | .08 | .041 | .0007 | .03 | .056 |
| .3125 gauge.....     | .17 | .87 | .009 | .025 | .78 | .04 | .68 | .07 | .040 | .0007 | .03 | .055 |

<sup>1</sup> Added in mold.

MECHANICAL PROPERTIES

| Bars             | Brinell<br>hardness<br>number | YS<br>(p.s.i.) | TS<br>(p.s.i.) | Elonga-<br>tion,<br>inches |       | TS/<br>YP | Bend  |
|------------------|-------------------------------|----------------|----------------|----------------------------|-------|-----------|-------|
|                  |                               |                |                | 2-8                        | 1 x t |           |       |
| "As rolled"..... |                               | 2% offset..... | .....          | 2-8                        | 1 x t | .....     | ..... |
| .250 gauge.....  | 223/241                       | 81,600         | 119,730        | 14-21                      | 1.37  | 1 x t     | ..... |
|                  |                               | 84,600         | 119,310        | 19                         | 1.41  | .....     | ..... |
|                  |                               | 99,040         | 117,620        | 15                         | 1.18  | .....     | ..... |
| .3125 gauge..... | 212/229                       | 76,200         | 102,080        | 23-33                      | 1.34  | 1½ x t    | ..... |
|                  |                               | 86,980         | 103,820        | 19                         | 1.19  | .....     | ..... |
|                  |                               | 94,280         | 103,120        | 20                         | 1.09  | .....     | ..... |

CHARPY "V" IMPACT TEST DATA

[Ft.-lbs.-at temperature ° F.]

| Thickness   | RT        | 32       | 0       | -20     | -40     |
|-------------|-----------|----------|---------|---------|---------|
| .250".....  | 7.0/4.7   | 5.5/3.3  | 4.7/3.0 | 3.2/2.5 | 2.3/2.0 |
| .3125"..... | 28.0/12.3 | 15.0/7.6 | 8.8/5.8 | 4.5/3.5 | 4.5/3.0 |

The process taught by the present invention, in addition to or in combination with the chemistry, also contributes to the desirable characteristics obtained. In practice the alloy steel is provided in billet form, that is in a suit-

able form for rolling into bars, plates or sheets. The billets are heat soaked at about 2100 to 2300° F., preferably about 2150° F., prior to rolling. The billets are then rolled. Multiple stand rolling is carried out so that finishing rolling temperature of the product of the present invention can be about 200° to 300° lower than the finishing rolling temperatures employed with high tensile strength steels in the prior art. The finishing rolling temperature should be in the range of 1400° to about 1700° F.

After rolling the product is allowed to cool without quenching or forced cooling. Such cooling will ordinarily take place at a rate of about 5 to 10° per second at least through the major portion of the cooling depending on the shape and thickness of the final product.

Other advantages of the invention are inherent in the above description. It is understood that changes and modifications in the foregoing teachings can be made without departing from the spirit of the invention so that the scope of the invention is to be determined from the appended claims.

I claim:

1. A low carbon, 75,000 p.s.i. minimum yield strength alloy steel consisting essentially, by weight, of

| Percent, about           |
|--------------------------|
| Carbon .....             |
| Manganese .....          |
| Silicon .....            |
| Chromium .....           |
| Zirconium .....          |
| Boron .....              |
| Titanium about .15% max. |
| Columbium .....          |

and the balance iron with residual impurities.

2. A low carbon, 75,000 p.s.i. minimum yield strength alloy steel consisting essentially, by weight, of

| Percent         |
|-----------------|
| Carbon.....     |
| Manganese.....  |
| Silicon.....    |
| Chromium.....   |
| Zirconium.....  |
| Boron.....      |
| Titanium.....   |
| Columbium.....  |
| Phosphorus..... |
| Sulphur.....    |
| Copper.....     |
| Aluminum.....   |

and the balance iron.

3. A low carbon high tensile strength alloy steel suitable for welding and characterized by minimum tensile strength of 75,000 p.s.i. in the "as rolled" condition with-

out subsequent heat treatment consisting essentially, by weight, of

|                          | Percent, about |
|--------------------------|----------------|
| Carbon                   | .07-.20        |
| Manganese                | .75-1.15       |
| Silicon                  | .50-1.0        |
| Chromium                 | .50-.80        |
| Zirconium                | .05-.20        |
| Boron                    | .0005-.0025    |
| Titanium about .15% max. |                |
| Columbium                | .01-.06        |

and the balance iron with residual impurities.

## References Cited

## UNITED STATES PATENTS

|             |         |          |          |
|-------------|---------|----------|----------|
| 3,328,211   | 6/1967  | Nakamura | 75-126 F |
| 2,234,130   | 3/1941  | Selmi    | 75-128 Z |
| 5 2,858,206 | 10/1958 | Boyce    | 75-126 I |
| 3,216,823   | 11/1965 | Gulya    | 75-128 Z |
| 3,251,682   | 5/1966  | Yawata   | 75-126 I |

HYLAND BIZOT, Primary Examiner

U.S. CL. X.R.

75-126 G, 126 Z

UNITED STATES PATENT OFFICE  
CERTIFICATE OF CORRECTION

Patent No. 3,689,258 Dated September 5, 1972

Inventor(s) JOSEPH R. ZANETTI

It is certified that error appears in the above-identified patent and that said Letters Patent are hereby corrected as shown below:

Column 3, line 8, (Example #1), " 518" " should read -- 5 1/8" --; line 59, (Example #2) under the column "Bend", "1 1/2 x" should read -- 1 1/2 x t --; (Example #2), "CHARPY "V" IMPACT TEST DATA" should read as follows:

CHARPY "V" IMPACT TEST DATA  
[Ft.-lb. at temperature ° F.]

| Thickness                     | R/T       | 32       | 0       | -20     | -40     |       |
|-------------------------------|-----------|----------|---------|---------|---------|-------|
| .250" (.394X.197X2.165).....  | 7.0/4.7   | 5.5/3.3  | 4.7/3.0 | 3.2/2.5 | 2.3/2.0 | (L)   |
| .3125" (.394X.295X2.165)..... | 28.0/12.3 | 15.0/7.6 | 8.8/5.8 | 4.5/3.5 | 4.8/3.0 | ..... |

Signed and sealed this 1st day of May 1973.

(SEAL)

Attest:

EDWARD M. FLETCHER, JR.  
Attesting Officer

ROBERT GOTTSCHALK  
Commissioner of Patents